

1

2,802,786

## EMULSIFIABLE OIL COMPOSITION

John D. Oathout, Cranford, N. J., assignor to Esso Research and Engineering Company, a corporation of Delaware

No Drawing. Application June 18, 1954,  
Serial No. 437,875

17 Claims. (Cl. 252—33.3)

The present invention relates to an emulsifiable oil composition and particularly to a so-called soluble cutting oil such as is used in metal working operations.

This application is a continuation-in-part of application Serial No. 291,977, filed June 5, 1952, and now abandoned.

In the prior art the advantages of the so-called soluble or emulsifiable cutting oils have been widely recognized. Since these oils are emulsifiable with water they can be combined with various proportions of water to simultaneously lubricate and cool the tools and the metal parts which are being operated upon. The prior art has considered it essential to use certain types of emulsifying ingredients in relatively large proportions in order to secure good solubility or emulsifiability in various proportions of water. In general, it is desired that soluble cutting oils be compatible with proportions of 1 to 50 or more parts of water for each part of the oil composition. Hence, it is essential that the emulsifying agents be highly effective.

Most successful prior art compositions have employed substantial proportions of oil soluble petroleum sulfonates as the primary emulsifying or solubilizing agent. For example, sodium sulfonates obtained by treating mineral oils with concentrated or fuming sulfuric acid and neutralizing with sodium hydroxide or the like have been widely used in soluble oils. These oil soluble sodium petroleum sulfonates are in general demand for various purposes including detergents, lubricating oil additives and the like. They are relatively expensive and often in short supply. Commercial cutting oils commonly employ as much as 10 to 15% by weight, on a dry basis, of these sulfonates, proportions of 12-15% being particularly common. Hence, compositions of this type consume large quantities of the relatively scarce and expensive sulfonates. One object of the present invention is to replace these sulfonates with other much less expensive ingredients which give comparable or even superior results.

In a copending application, Serial No. 291,978, and now abandoned, filed contemporaneously with Serial No. 291,977, there is disclosed an improved soluble oil composition of a related type. Therein certain naphthenic acid soaps and other ingredients are derived from pipe still bottoms, i. e. residues from acid-treated and caustic-treated distillation operations are combined with sulfonates or rosin soaps, etc. to make a relatively inexpensive product of excellent emulsion characteristics.

In the present case, another inexpensive residue material from a different type of refining operation is utilized as an important ingredient. In the extraction of undesired naphthenic acids and related materials from lubricating oil, especially Colombian or Coastal stocks of high naphthenic content, one process involves the use of aqueous solutions of an aromatic sulfonate material rich in sodium xylene and/or toluene sulfonates, etc. and sodium hydroxide, which is called "Napex" solution. The aromatic sulfonate material used in this solution is

2

obtained as the neutralized sulfuric acid extract from the finishing of toluene and xylene streams with concentrated sulfuric acid. This extract normally contains, in addition to aromatic sulfonates, small proportions of 5 inorganic salts, caustic and organic sulfates and a major proportion of water. The most desirable fresh "Napex" solutions used to extract naphthenic base stock contain about 20 to 30 wt. percent of toluene and xylene sulfonates, 10 to 15% inorganic salts, principally sodium 10 sulfate, 0.5-5 wt. percent of caustic soda and 50 to 70 wt. percent of water.

More specifically, the lubricating oil distillates are treated with about 15-25 lbs. of strong sulfuric acid of about 98% strength per barrel of oil. A sludge is formed 15 which is allowed to separate. The acid oil layer is subsequently extracted with about 4-10 bbl. per 100 bbl. of oil, of a "Napex" solution of the type described above, e. g. a solution containing about 26% of sodium toluene and xylene sulfonates, about 12.5% of inorganic salts, 20 about 3.5% of free sodium hydroxide and about 58% of water. The oil—"Napex" mixture is preferably heated to about 125°-210° F., for example by steam blowing, and allowed to settle, at which point the spent "Napex" solution containing dissolved naphthenates and sulfonates 25 and some oil separates as the bottom layer or extract and is drawn off. The "Napex" solution may be recirculated one or more times but eventually it becomes loaded with sludge or otherwise spent. The spent "Napex" solution is then cooled, treated with 1-2 volumes 30 of water and allowed to settle. An organic upper layer is separated. Alternately, the water contained in the spent "Napex" solution may be removed therefrom by flashing or distilling and any solid inorganic material remaining in the organic material may be removed by 35 decanting or filtering.

The organic material so separated, which normally contains about 3-20 wt. percent of water-soluble low molecular weight sulfonates, may be used for the purposes of the present invention. If it is desired further 40 to purify this material, it may be acidified to a pH of 3 and then treated with aqueous sodium hydroxide while removing water which separates upon acidification and alkalization. Such purification treatment may reduce the low molecular weight sulfonate content of the 45 "Napex" solution to less than 3 wt. percent. The sodium soap concentrate thus formed is blown with hot air until the concentrate is substantially free of water.

The "Napex" solution so obtained is a relatively heavy sludge which contains relatively large proportions of 50 soaps, including substantial proportions of naphthenates and some sulfonates. These sludge or spent materials are used as emulsifying agents in soluble oils. They may be used also in combination with conventional (and relatively expensive) sulfonates such as oil-soluble petroleum 55 sulfonates, or they may, according to one aspect of the invention, be used with other soaps, such as the alkali metal rosin soaps, e. g. the potassium or sodium rosinates sold commercially by Hercules Powder Company under the trade names "Dresinate 92," "Dresinate 93," etc. 60 Alternatively the sulfonates, rosinates, and other soap and non-soap emulsifiers, including the partial esters of polycarboxylic acids and other non-ionic emulsifiers may be used with the spent "Napex" type solutions in various combinations.

65 The invention, therefore, has the advantage of replacing a relatively expensive ingredient (sodium or other oil-soluble high molecular weight sulfonate) hitherto deemed essential with a material containing substantial proportions of water-soluble aromatic low molecular weight sulfonates, which has previously been considered largely a waste, with eminently satisfactory results. In some cases

it may be desirable to retain some of the relatively expensive sulfonate, especially where rust prevention in machined steels and other ferrous metals is of paramount importance. Hence, proportions of 2-25% by weight of the spent "Napex" type product may be used in mineral base oil of lubricating grade, along with 1-10% of other soap-type emulsifying agents. The "Napex" product will have a soap content, primarily sodium naphthenate and high and low molecular weight sulfonates, of 25-75% by weight. In general, the naphthenate soap content is between 10 and 50% of the spent "Napex" product, so that an oil containing 2-25% of the spent "Napex" will contain about 0.2-12 or 13% of sodium naphthenates. Rosin soaps, where used, may be present in approximately equal proportions, i. e. 1-5 or 10% by weight of the soluble oil composition. The total sulfonates present in the spent "Napex" may comprise about 5-50% of the spent "Napex" or about 0.1-15% of the oil product. In typical cases which will be illustrated below, the high-molecular weight, oil-soluble sulfonates (about 350-500 mol. wt.) made up about  $\frac{1}{6}$ - $\frac{1}{2}$  of the soap content of the spent "Napex." The content of low molecular weight water-soluble sulfonates may be about 0.5-20% by weight of the spent "Napex." Normally the weight ratio of naphthenates to high molecular weight sulfonates is about 0.5-5:1. In all cases, however, requirements for the usual expensive oil-soluble petroleum sulfonate ingredients are materially reduced and good use is made of a product formerly considered quite worthless. As in said copending application, a balancing agent may be needed.

The invention will be more fully understood by reference to specific examples:

#### Example I

Four samples of spent "Napex" product, considered representative of normal production at a large refinery, were taken. Two of these samples (a) and (a') were taken from the refining of a Coastal oil of about 1,000 S. S. U. viscosity at 100° F., and two samples (b) and (b') from the refining of another Coastal oil of about 100 S. S. U. at 210° F.

Samples (a') and (b') were spent "Napex" product obtained as follows. The Coastal distillates were treated with approximately 20 lbs./bbl. of 98% black sulfuric acid. After removal of sludge the acid oil was extracted with about 6 bbls. of the fresh "Napex" solution, specifically described above, per 100 bbls. of oil. The oil-Napex mixture was heated to 190° F. by blowing with steam. The spent "Napex" solution was then allowed to separate as the bottom layer. On cooling to about 90° F. a water layer separated, which was discarded. The organic layer was blown with air to remove water. About 12 bbls. of spent "Napex" product were recovered per 100 bbls. of oil treated.

Samples (a) and (b) were spent "Napex" products obtained as described above which were, prior to air blowing, further acidified with sulfuric acid to a pH of 3 followed by alkalizing with sodium hydroxide to a pH of 10.

These four samples had the following composition:

|                                                          | (a)   | (a')  | (b)   | (b')  |
|----------------------------------------------------------|-------|-------|-------|-------|
| Percent Oil                                              | 47.0  | 72.0  | 65.2  | 42.0  |
| Percent Inorganic Salt                                   | 3.7   | 0.2   | 5.3   | 1.7   |
| Percent Total Soap                                       | 48.1  | 28.0  | 29.5  | 48.0  |
| Combining Wt. of Soap (as Na)                            | 422.0 | 405.0 |       |       |
| Percent Naphthenate                                      | 22.8  | 19.6  | 10.5  | 15.8  |
| Combining Wt. of Naphthenate (as Na)                     | 495.0 | 460.0 | 540.0 | 545.0 |
| Percent High Molecular Weight Sulfonate                  | 22.8  | 4.7   | 15.6  | 16.3  |
| Combining Wt. of High Molecular Weight Sulfonate (as Na) | 417.0 | 393.0 | 400.0 | 447.0 |
| Percent Low Molecular Weight Sulfonate                   | 0.7   | 3.4   | 2.0   | 17.2  |
| Combining Wt. of Low Molecular Wt. Sulfonate (as Na)     | 231.0 | 103.0 | 200.0 | 135.0 |

Three blends of products (a) and (b) were prepared. The following were prepared from product (a):

|                                              | Blend No.                                             | I            | II           | III |
|----------------------------------------------|-------------------------------------------------------|--------------|--------------|-----|
| Composition, Wt. Percent:                    |                                                       |              |              |     |
| "Napex"                                      | 10.4                                                  | 15.6         | 21.0         |     |
| Mineral Lube Oil, 45 S.S.U.                  | 84.6                                                  | 79.4         | 75.0         |     |
| vis. at 210° F.                              |                                                       |              |              |     |
| Diethylene glycol                            | 3.0                                                   | 3.0          | 3.0          |     |
| Water                                        | 2.0                                                   | 1.0          | 0.5          |     |
| Triethanolamine                              | 5.0                                                   | 7.5          | 10.0         |     |
| Percent "Napex" Soap in Blend                |                                                       |              |              |     |
| Emulsibility                                 | Blend could not be balanced satisfactorily, rejected. | Fair-Good.   | Fair.        |     |
| Emulsion Separation: 10/1 Tap Water, 24 hrs. |                                                       | 1 cc. Cream. | 1 cc. Cream. |     |
| Rust Rating: 40/1 Emulsion                   |                                                       | 1,1          | 1,1          |     |

On the basis of emulsibility and blend appearance, blend II was selected as the best of these three.

A similar study of "Napex" sample (b), blended at concentrations which resulted in the same soap concentrations as reported above (5, 7.5, and 10%) gave similar results: the 5% (soap basis) blend could not be brought into balance, and was rejected. The 7.5% soap blend was best, showing fair-good emulsibility, no blend separation, and a 40/1 emulsion resulted in a rust rating of 0. Emulsion stability was rather poor showing a separation of 25 cc. of cream after 24 hours. This probably may be corrected by more careful balancing with triethanolamine and coupling agents. The blend containing 10% "Napex" soap required 34% "Napex" concentrate in its blend, with the result that the blend was too viscous to be satisfactory.

Incorporation of 4.0 wt. percent "Dresinate 93," a liquid potassium rosinate (containing 12.5% diethylene glycol) manufactured by the Hercules Power Company, in the blends containing 5% "Napex" soaps resulted in marked improvement in these blends with respect to emulsibility and emulsion stability. Rust ratings were somewhat inferior, however.

On the basis of the data obtained in the screening tests, larger soluble oil samples were prepared, and studied more fully. The compositions of these blends, and laboratory results are as follows:

|                                 | Blend No.        | IV             | V    | VI    |
|---------------------------------|------------------|----------------|------|-------|
| Composition, Wt. Percent:       |                  |                |      |       |
| "Napex" (a)                     | 15.6             | 15.6           |      | 16.80 |
| "Napex" (b)                     |                  |                |      | 2.98  |
| "Dresinate 93"                  |                  |                |      | 2.98  |
| Diethylene Glycol               | 4.0              | 3.0            |      | 2.98  |
| Water                           | 2.0              | 1.0            |      | 1.98  |
| Mineral oil of 45 SSU Viscosity | 78.4             | 79.4           |      | 74.10 |
| Triethanolamine                 | ( <sup>1</sup> ) | 1.0            |      | 1.20  |
| Emulsibility                    |                  | Good-Excellent | Good |       |

<sup>1</sup> This blend appeared cloudy at all times and could not be balanced satisfactorily. Rejected.

|                                             | Blend No.               | V                                | VI   |
|---------------------------------------------|-------------------------|----------------------------------|------|
| Emulsion Separation: 10/1 Tap Water 24 hrs. | Trace Oil, Trace Cream. | 2 cc. fine cream.                |      |
| Blend Stability:                            |                         | No Separation                    |      |
| 2 Weeks at Room Temperature                 |                         | No Separation                    |      |
| 1 Week at 35° F                             |                         |                                  |      |
| Rust Rating:                                |                         |                                  |      |
| 40/1 Emulsion                               |                         | 2-3, 2                           | 2, 2 |
| Staining                                    |                         | Moderate Stain in Emulsion Layer |      |
| CSC, 1 10/1 Emulsion: 3 hrs. at 122° F.     | J-3 <sup>2</sup>        | J-3 <sup>2</sup>                 |      |

<sup>1</sup> Copper Strip Corrosion.

<sup>2</sup> Scale: J-1 to J-10; J-3 denotes very light stain.

Additional blends were prepared from "Napex"-solution (b') and tested as indicated in the table below.

| Blend No.                                    | VII  | VIII          | IX     | X           |
|----------------------------------------------|------|---------------|--------|-------------|
| Composition, Wt. Percent:                    |      |               |        |             |
| "Napex" (b')                                 | 18.8 | 10.4          | 14.8   | 18.9        |
| Mineral Lube Oil, 45 SSU @ 210° F.           | 75.5 | 83.4          | 79.2   | 75          |
| Isopropyl Alcohol                            | 1.9  |               |        |             |
| "Dresinate 93"                               | 3.8  | 6.2           | 6.0    | 5.7         |
| Percent "Napex" Soap in Blend                | 9.0  | 5.0           | 7.1    | 9.1         |
| Emulsibility                                 | Fair | Fair          | Fair   | Fair        |
| Emulsion Separation: 10/1 Tap Water, 24 hrs. | Good | 2 cc.         | Trace  | 5 cc.       |
|                                              |      | Coarse Cream. | Cream. | Fine Cream. |

It will be noted that these blends which contained about equal proportions of oil-soluble high molecular weight sulfonates and water-soluble low molecular sulfonates and about equal proportions of naphthenates and high molecular weight oil-soluble sulfonates had commercially acceptable emulsification characteristics. This result was obtained without further balancing the blends in the manner described above. The emulsibility and emulsion separation of these blends may be easily changed from a rating of "Fair" and "Good," respectively, to a rating of "Good-Excellent" and equivalent ratings, by balancing the blends as indicated above.

From these data, it appears that blends incorporating "Napex" concentrates with or without "Dresinates" compare favorably in properties with competitive brands of soluble oils. The "Napex" soluble oils appear to be superior to some formulations with respect to emulsibility (ease of emulsion formation) and blend stability.

Blends of the type described above not only have good emulsification properties in various proportions of water but they also have good load carrying properties.

The triethanolamine used in the blends mentioned above was employed as a balancing agent. In some cases, it might be necessary to use an acid, e. g. oleic or related fatty acid instead of the amine, to bring the pH value to the desired level or about 7.2 to 8.5, as explained more fully in the copending application filed simultaneously with Serial No. 291,977 and mentioned above (Serial No. 291,978).

Also, as mentioned in said copending application, it is desirable to use as a coupling or blending agent an aliphatic alcohol, preferably diethylene glycol, in proportions up to 5%, preferably about 1% to 4%, based on the weight of the oil blend. Other alcohols, such as isopropyl, may be used but diethylene glycol is somewhat superior to facilitate blending the oil with water.

The present invention contemplates also the preparation of a blending or emulsifying agent per se. In such cases, 40-75% of the spent "Napex" solution may be combined with 25-55% of another soap of good emulsifying properties, e. g. rosin soap. It is preferred to use at least 20% of rosin soap where the sulfonate content of the spent "Napex" solution is low but it may be omitted altogether where the sulfonate content of the "Napex" approaches half of its total soap content. Even in such cases it may be desirable to use up to 3% of such soap, as in blend VI, above.

Diethylene glycol or other assisting agents may be used in proportions up to 10% or more and when needed, an alkanolamine or a fatty acid is employed to bring the pH value to the desired level as previously explained. A small amount of water added to the oil, e. g. (up to 3% or so) aids in emulsification.

It will be understood that conventional modifiers may be used also, such as rust inhibitors (e. g. phosphites, chromites, etc.), extreme pressure agents, oiliness agents, etc., as will be obvious to those skilled in the art. In some cases synthetic lubricating oils, e. g. diesters, complex esters, etc. of appropriate viscosity, as well as synthetic hydrocarbon oils may be used as a part or all of

the oil base. The viscosity of the oil may vary over a wide range, e. g. from 35-1000 S. S. U. at 210° F., the lower part of this range, up to 120 S. S. U. or so, usually being more desirable.

- 5 What is claimed is:
1. An emulsifiable metal working oil composition comprising a major proportion of a lubricating oil and a minor proportion sufficient to render said oil emulsifiable, of a sulfonate-naphthenate material obtained by separating an organic layer from the extract formed in the extraction of mineral base lubricating oil of high naphthenic content with an aqueous solution of water-soluble sulfonate material selected from the group consisting of sodium xylene sulfonate, sodium toluene sulfonate and mixtures thereof, and sodium hydroxide.
  2. A composition as claimed in claim 1 in which said naphthenic lubricating oil is an oil treated with strong sulfuric acid prior to said extraction.
  3. A composition as claimed in claim 1 which contains about 2-25 wt. percent of said material.
  4. A composition as claimed in claim 1 in which said material contains a total of about 25-75 wt. percent of sodium sulfonates and naphthenates, based on said material.
  5. A composition as claimed in claim 1 in which said material contains about 10-50 wt. percent of sodium naphthenates, based on said material.
  6. A composition as claimed in claim 1 in which said material contains about 0.5-20 wt. percent of low molecular weight water-soluble sulfonates selected from the group consisting of sodium xylene sulfonate, sodium toluene sulfonate and mixtures thereof, based on said material.
  7. A composition as claimed in claim 1 in which the weight ratio of naphthenates to high molecular weight oil-soluble sulfonates in said material is about 0.5-5:1.
  8. A composition as claimed in claim 1 in which said material contains about 0.1-15 wt. percent of total sulfonates, based on said composition.
  9. A composition as claimed in claim 1 in which about  $\frac{1}{6}$ - $\frac{1}{2}$  of the total naphthenate and sulfonate content of said material is high molecular weight oil-soluble sulfonate.
  10. A composition as claimed in claim 1 which contains about 1-10% by weight of rosin soap, based on said composition.
  11. A composition as claimed in claim 1 which contains about 1-4 wt. percent of a coupling agent selected from the group consisting of glycols, aliphatic alcohols and water.
  12. An emulsifying agent for lubricating oils comprising about 25 to 55% by wt. of a soap having emulsifying properties and about 40-75% by weight of a sulfonate-naphthenate material obtained by separating an organic layer from the extract formed in the extraction of mineral base lubricating oil of high naphthenic content with an aqueous solution of water-soluble sulfonate material selected from the group consisting of sodium xylene sulfonate, sodium toluene sulfonate and mixtures thereof, and sodium hydroxide.
  13. An oil composition of the approximate formula by weight:
- 65 74-85% mineral base lubricating oil
- 10-21% of a sulfonate-naphthenate material obtained by separating an organic material from the extract formed in the extraction of mineral base lubricating oil of high naphthenic content with an aqueous solution of water-soluble sulfonate material selected from the group consisting of sodium xylene sulfonate, sodium toluene sulfonate and mixtures thereof, and sodium hydroxide, said material containing about 0.5-20 wt. percent of low molecular weight water-soluble sulfonates based on said material and naphthenates and

high molecular weight oil-soluble sulfonates in a weight ratio of about 0.5-5:1  
 3-4% diethylene glycol  
 0.5-2% water  
 0.5-1.5% triethanolamine

14. A composition as claimed in claim 13 which contains about 1-10% of alkali metal soap of rosin acids.

15. An oil composition of the approximate formula by weight:

75-84% mineral lubricating oil  
 10-20% of a sulfonate-naphthenate material obtained by separating an organic material from the extract formed in the extraction of mineral base lubricating oil of high naphthenic content with an aqueous solution of water-soluble sulfonate material selected from the group consisting of sodium xylene sulfonate, sodium toluene sulfonate and mixtures thereof and sodium hydroxide, said material containing about 0.5-20 wt. percent of low molecular weight water-soluble sulfonates, based on said material and naphthenates and high molecular weight oil-soluble sulfonates in a weight ratio of about 0.5-5:1  
 3-6% of alkali metal soap of rosin acids

15  
 20

16. A composition as claimed in claim 15 which contains about 1-4% of isopropyl alcohol.

17. An emulsifiable metal working oil composition comprising a major proportion of a lubricating oil and a minor proportion sufficient to render said oil emulsifiable, of a sulfonate-naphthenate material obtained by adding water to the extract formed in the extraction of a mineral base lubricating oil of high naphthenic content with an aqueous solution of a water-soluble sulfonate material selected from the group consisting of sodium xylene sulfonate, sodium toluene sulfonate and mixtures thereof, and sodium hydroxide, and recovering said sulfonate-naphthenate material as an organic layer of said water-diluted extract.

References Cited in the file of this patent  
 UNITED STATES PATENTS  
 2,340,035 Zimmer et al. ----- Jan. 25, 1944